

## UNITED STATES PATENT OFFICE

HAROLD GEORGE LACELL, DECEASED, LATE OF FINCHLEY, LONDON, ENGLAND, BY ELIZA LACELL, EXECUTRIX, OF FINCHLEY, LONDON, ENGLAND

## PROCESS FOR THE DEHYDRATION OF MAGNESIUM CHLORIDE

No Drawing. Application filed March 31, 1930, Serial No. 440,637, and in Germany April 5, 1929.

This invention is based on the surprising discovery that by adding a relatively small amount of hydrated magnesium chloride to a considerable liquid mass of magnesium chloride which has been substantially completely dehydrated and is sufficiently hot, the water of hydration became vaporized and only a small amount of the chloride was converted into magnesium oxide, contrary to what would be expected.

The present invention relates to a process for the dehydration of hydrated magnesium chloride, which consists in the use of the heat capacity of a relatively large mass of magnesium chloride which is practically anhydrous, in order to rapidly raise the temperature of a relatively small amount of magnesium chloride to be dehydrated, thus rapidly vaporizing the water without forming any great quantity of oxide.

Preferably, the mass of magnesium chloride is heated by electricity which disengages heat within the said mass, using alternating current, high frequency induction currents, etc.

It is preferable to add to the magnesium chloride a small amount of potassium chloride, and good results have been obtained with one molecule of potassium chloride for two of magnesium chloride. This lowers the temperature of fusion of the bath, and the dehydration appears to be furthered.

The process may be carried out as follows. An alternating current is sent through a bath of practically anhydrous magnesium chloride and potassium chloride in the proportion of at least one molecule of potassium chloride for two of magnesium chloride, thus heating the bath to at least 500° C. then adding hydrated magnesium chloride at stated intervals to the hot mass. Each addition of the hydrated material causes a rather violent boiling up, due principally to the disengagement of the water contained in the hydrated magnesium chloride so added. The amount of magnesia produced is always small. The steam thus given off must be at once removed from contact with the bath, for instance by producing a slight suction

on the bath, the latter being held in a closed vessel.

It appears that the important point consists in the fact of suddenly raising the temperature of the hydrated magnesium chloride in such manner that the water will be rapidly given off, and thus will not act upon the resulting magnesium chloride.

It is to be noted that the presence of the potassium chloride which is added causes no difficulties in the subsequent use of the magnesium chloride in the electrolytic vats for the production of magnesium.

Further, it is entirely feasible to add the magnesium chloride to be dehydrated, in a continuous manner, provided the amount of chloride added is not sufficient to cause an excessive cooling of the whole mass. The added amount of the magnesium chloride to be dehydrated will be greater as the quantity of heat furnished to the bath is greater, and in practice it is advisable to maintain the temperature of the mass as uniform as possible by suitable additions and an adequate heating.

## What is claimed is:

1. A process for the dehydration of magnesium chloride, which comprises gradually adding, to a relatively large mass of molten anhydrous magnesium chloride, relatively small quantities of hydrated magnesium chloride, thus causing a rapid vaporization of the water of hydration and thereby preventing the formation of magnesium oxide.

2. Process in conformity to the claim 1, characterized by the fact that the temperature of the melted mass is maintained at about 500° C., and between relatively narrow limits by regulating the heating and by regulating the quantities of the hydrated chloride of magnesium added.

3. Process in conformity to the claim 1, characterized by the fact that the melted mass is heated by heat generated electrically within the body of the mass.

4. Process in conformity to the claim 1 characterized by the fact of adding potassium chloride to the mass of anhydrous magnesium chloride in order to lower the melting point.

5. Process in conformity to the claim 1

characterized by the fact that the liquid mass is maintained during such process under a partial vacuum to facilitate the vaporizing and removal of the water of hydration.

5 6. A process of dehydration of magnesium chloride consisting of maintaining a relatively great mass of anhydrous material rich in magnesium chloride in a molten state, and of adding to that mass relatively smaller quantities of a material containing a hydrated magnesium chloride.

7. A process of dehydration of magnesium chloride consisting of maintaining an anhydrous mass relatively rich in magnesium chloride in a molten state, by a heating thereof without action on the composition of said chloride, and adding to that mass relatively smaller quantities of material rich in hydrated magnesium chloride.

15 8. A process of dehydration of magnesium chloride consisting of maintaining a relatively great mass of material rich in magnesium chloride in a molten state by heating the said mass to about 500° C., and adding to that mass relatively smaller amounts of a mass containing hydrated magnesium chloride.

9. A process of dehydration of magnesium chloride consisting of maintaining a relatively large anhydrous mass of material which is stable at a high temperature and which is rich in magnesium chloride, in a molten state by internally heating the same to about 500° C., and by adding to this mass relatively smaller quantities of material containing hydrated magnesium chloride.

30 10. A process of dehydration of magnesium chloride consisting of maintaining a mass of anhydrous material rich in magnesium chloride in a molten state, by heat generated within said mass of material, and adding to this mass relatively smaller amounts of a material rich in hydrated magnesium chloride.

45 11. A process of dehydration of magnesium chloride which comprises maintaining a relatively great quantity of substantially anhydrous material rich in magnesium chloride, at a temperature at which such material is molten, and while under a pressure below normal atmospheric, and adding to that mass relatively smaller quantities of a material rich in hydrated magnesium chloride.

In testimony whereof I have signed this specification.

55 ELIZA LACELL,  
*Executrix of Harold George Lacell, Deceased.*